# EUROPEAN PATENT SPECIFICATION

(11) **EP 3 147 379 B1**
(45) Date of publication and mention of the grant of the patent: **05.08.2020**
(21) Application number: 15795946.1
(22) Date of filing: 15.05.2015
(51) Int. Cl.: C22C 38/02, C22C 38/04, C22C 38/16, C22C 38/18, C22C 38/20, C22C 38/38, C22C 38/58, C21D 8/02

(54) **THICK STEEL PLATE**
DICKE STAHLPLATTE
PLAQUE D'ACIER ÉPAISSE

(30) Priority: 22.05.2014 JP 2014106307; 20.04.2015 JP 2015086047
(43) Date of publication of application: 29.03.2017
(62) Divisional of application: 19220022.8
(73) Proprietor: Kabushiki Kaisha Kobe Seiko Sho (Kobe Steel, Ltd.), Kobe-shi, Hyogo 651-8585 (JP)
(72) Inventor: SANDAIJI, Yusuke, Kobe-shi Hyogo 651-2271 (JP); KINEFUCHI, Masao, Kobe-shi Hyogo 651-2271 (JP); KAWANO, Haruya, Kakogawa-shi Hyogo 675-0137 (JP)
(74) Representative: Müller-Boré & Partner Patentanwälte PartG mbB
(86) International application number: PCT/JP2015/064099
(87) International publication number: WO 2015/178320

(56) References cited:
- EP-A1- 2 006 407
- EP-A1- 2 157 203
- WO-A1-2015/041118
- JP-A- S6 415 319
- JP-A- S6 415 319
- JP-A- 2007 197 823
- JP-A- 2007 197 823
- JP-A- 2008 297 575
- JP-A- 2008 297 575
- JP-A- 2012 172 256
- JP-A- 2012 172 256

## Description

The present invention relates to steel plates. Specifically, the present invention relates to a steel plate that is mainly used as materials for structures such as ships buildings, bridges, and construction machinery, has a tensile strength of 490 MPa to less than 650 MPa, and offers excellent fatigue properties.

With upsizing, large structures such as ships, buildings, bridges, and construction machinery require still better reliability of their structural components, because such larger structures, if suffering from breakage, may receive larger damage. It has been known that most of breakages in large structures is caused by fatigue fracture. As possible solutions to this, various techniques for resisting fatigue fracture have been developed. However, there are not a few cases where fatigue fracture causes breakage of such a large structure, even now.

In general, portions of large structures susceptible to fatigue damage have been protected from fatigue fracture by schemes such as designing of the portions to have such a shape as to less cause stress concentration, and use of high-strength steel plates. However, the resulting structures obtained according to the schemes cause higher production cost due to a higher number of steps or due to the use of more expensive steel plates. Accordingly, demands are made to provide a technique for allowing a steel plate itself to have better fatigue properties. In general in steel plates, it is known that fatigue strength, in particular fatigue limit, is in proportional to tensile strength, and a steel plate having a high fatigue limit to tensile strength ratio is considered as a steel plate having excellent fatigue properties, where the fatigue limit to tensile strength ratio is calculated by dividing the fatigue limit by the tensile strength.

Many researches have been performed so as to offer better fatigue properties. For example, Nonpatent Literature (NPL) 1 presents how various influencing factors affect fatigue strength. The literature mentions that solid-solution strengthening, precipitation strengthening, grain refinement, and second phase strengthening contribute to better fatigue properties, but dislocation hardening less contributes to better fatigue properties, because the dislocation hardening is attended with increase in moving dislocations. The fatigue fracture process can be divided into a process (1) and a process (2). In the process (1), a load is repeatedly applied, and, finally, cracks are generated. In the process (2), the generated cracks grow and lead to rupture (breakage). Of the above-mentioned factors for better fatigue properties, solid-solution strengthening, precipitation strengthening, and grain refinement are considered to be effective in the process (1), because restrainment of accumulation of dislocations is effective in this process. In contrast, grain refinement and second phase strengthening are considered to be effective in the process (2), because elimination or minimization of crack propagation is effective in this process.

Patent Literature (PTL) 1 proposes a technique in which the steel is controlled to have a two-phase microstructure including fine ferrite and hard martensite, and the difference in hardness between the two phases is specified to be 150 or more in terms of Vickers hardness. The technique is intended to lower the crack propagation rate and to contribute to a longer fatigue life after crack initiation.

PTL 2 proposes a technique for lowering the crack propagation rate by allowing the steel to have a mixed microstructure including fine ferrite and bainite. This technique is expected to offer longer fatigue life after crack initiation also in fatigue fracture. However, the technique lacks consideration of fatigue properties before crack initiation at all.

PTL 3 proposes a technique of allowing carbides to precipitate in ferrite phase so as to offer higher fatigue strength. This literature, however, lacks description about fatigue properties after crack initiation. In addition, the technique in PTL 3 targets thin steel sheets and gives no consideration to toughness and other properties necessary for large structures at all.
NPL 1: Abe et aL, "Tetsu-to-hagane", Vol. 70 (1984), No. 10, pp. 1459-1466
PTL 1: Japanese Unexamined Patent Application Publication (JP-A) No. Hei10-60575
PTL 2: JP-A No. 2011-195944
PTL 3: JP-A No. 2009-84643

Furthermore, JP 2012 172256 A discloses a low yield ratio high strength hot rolled steel sheet which shall have a low temperature toughness, as well as a method for manufacturing the same.

The present invention has been made under these circumstances and has a main object to provide a steel plate having excellent fatigue properties.

Other objects of the present invention will be apparent from the description below.

The present invention has achieved the objects and provides a steel plate as follows. The steel plate contains C in a content of 0.02 to 0.10 mass percent, Mn in a content of 1.0 to 2.0 mass percent, Nb in a content of greater than 0 mass percent to 0.05 mass percent, Ti in a content of greater than 0 mass percent to 0.05 mass percent, Al in a content of 0.01 to 0.06 mass percent, Cu in a content of 0.1 to 0.6 mass percent, and Ni in a content of greater than 0 mass percent to 0.6 mass percent, where a ratio [Ni]/[Cu] of the Ni content [Ni] to the Cu content [Cu] is 0.5 to less than 1.2, optionally comprising Si in a content of 0.1 to 0.6 mass percent, where the total content of Si and Cu is 0.3 mass percent or more, optionally comprising, in chemical composition, at least one selected from the group consisting of
(b) at least one element selected from the group consisting of V in a content of greater than 0 mass percent to 0.5 mass percent; Cr in a content of greater than 0 mass percent to 1.0 mass percent or less; and Mo in a content of greater than 0 mass percent to 0.5 mass percent; and
(c) B in a content of greater than 0 mass percent to 0.005 mass percent, with the remainder consisting of iron and inevitable impurities. The microstructure of the surface layer of the steel plate includes at least one of ferrite and upper bainite in a total fraction of 80 area percent to 100 area percent, wherein, of the microstructure of the surface layer, the remainder microstructure excluding the ferrite and the upper bainite optionally has a fraction of martensite-austenite constituent of 0 area percent to 5 area percent. Grains of the at least one of ferrite and upper bainite have an effective grain size of 2 µm to 10.0 µm. Of the microstructure of the surface layer, grains of the remainder microstructure excluding the ferrite and the upper bainite have an average equivalent circle diameter of 0.5 µm to 3.0 pm. The steel plate has a dislocation density ρ of 5.0×10¹³ m⁻¹ to 2.5× 10¹⁵ m⁻¹, as determined by X-ray diffractometry.

As used herein, the term "average equivalent circle diameter" refers to an average of "equivalent circle diameters" of grains of a phase in question, where the "equivalent circle diameter" refers to the diameter of a grain of the phase in terms of a circle having an equivalent area to the grain.

The steel plate according to the present invention preferably further contains at least one selected from the group consisting of (b) and (c) below. The steel plate may have further improved property or properties depending on the type of an element to be contained. Specifically, the steel plate preferably further contains at least one selected from the group consisting of
(b) at least one element selected from the group consisting of V in a content of greater than 0 mass percent to 0.5 mass percent, Cr in a content of greater than 0 mass percent to 1.0 mass percent or less, and Mo in a content of greater than 0 mass percent to 0.5 mass percent; and
(c) B in a content of greater than 0 mass percent to 0.005 mass percent.

The steel plate according to the present invention also preferably has a bainite transformation start temperature Bs of 640°C or higher, where the bainite transformation start temperature is calculated from the chemical composition according to Expression (1): $Bs \left(°C\right) = 830 - 270 \left[C\right] - 90 \left[Mn\right] - 37 \left[Ni\right] - 70 \left[Cr\right] - 83 \left[Mo\right]$ where [C], [Mn], [Ni], [Cr], and [Mo] represent contents (in mass percent) respectively of C, Mn, Ni, Cr, and Mo.

Advantageous effects of the present invention as disclosed in the description will be briefly described as follows. Specifically, the present invention can practically provide steel plates that have excellent fatigue properties.
Fig. 1 depicts schematic explanatory views of a steel plate according to the present invention;
Fig. 2 depicts schematic explanatory views of a test specimen used in measurements of fatigue properties;
Fig. 3 depicts schematic explanatory views of a compact tension test specimen used in crack propagation rate measurement; and
Fig. 4 depicts conceptual diagrams illustrating grain boundaries, KAM, and GAM.

The inventors of the present invention made investigations of the total life of steel plates leading up to fatigue fracture and particularly of proportions of the prior-stage life leading to crack initiation and of the subsequent-stage life from crack initiation leading up to rupture. As a result, the inventors found that the prior-stage life leading to crack initiation occupies about one half of the total life leading up to fatigue fracture; and that the prior-stage life leading to crack initiation occupies a larger proportion with a decreasing stress level and a resulting increasing total life. The results indicate that increase of the total life leading up to fatigue fracture requires not only better fatigue properties after crack initiation, but also better fatigue properties leading to crack initiation. In particular, at around the fatigue limit, increase in prior-stage life is considered to be effective because the prior-stage life leading to crack initiation tends to occupy a larger proportion of the total life.

The inventors made various investigations on conditions for a longer prior-stage life. As a result, the inventors found that a steel plate as follows can have a longer prior-stage life, and consequently have a longer total life leading up to fatigue fracture. This steel plate is appropriately controlled in the chemical composition, and conditions typically on the fraction(s) of principal phase(s), the effective grain size of grains of the phase(s), the average equivalent circle diameter of the remainder microstructure excluding the principal phase(s), and the dislocation density ρ as determined by X-ray diffractometry. The present invention has been made based on these findings.

The present invention will be illustrated below. The inventors made investigations on various steel plates about how elements to be added affect the fatigue strength. Consequently, the inventors found that the addition of Si and/or Cu significantly improves the fatigue strength. In general, moving dislocations, which move by repeated stress, move irreversibly due typically to cross slip, and this causes fatigue cracking. It is known that the dislocations form a cell structure in this process. The inventors found that the addition of Si and/or Cu in a total amount of 0.3 mass percent or more restrains the cell structure formation.

Detailed observations demonstrate that these elements do not form precipitates and are not noticeably dissolved as solutes typically in carbides present in steel plates, but are probably dissolved and present as solutes in the matrix. Specifically, it is considered that a steel plate can have a longer fatigue life up to (prior to) crack initiation by allowing these elements to be dissolved and present as solutes sufficiently in the matrix to thereby restrain the irreversible movements of dislocations. The inventors also found that other elements to be added, such as Mn and Cr, do not noticeably offer the effect of restraining dislocations from forming a cell structure, but rather lower the transformation temperature to cause the formation of lower bainite, which has a high dislocation density; and that such other elements to be added do not so much improve fatigue strength as compared with static strength.

In addition, the inventors prepared various steel plates under different rolling conditions and made investigations on how the rolling conditions affect the mechanical properties and fatigue strength of the resulting steel plates. As a result, the inventors found that steel plates, when caused to have a higher dislocation density typically by rapidly cooling the steel plates down to a low temperature, or by applying compression reduction (performing rolling) at a temperature equal to or lower than the Ar₃ transformation temperature, have higher static strength such as yield stress and tensile strength, but have not so higher fatigue strength as compared with the static strength, and have a lower fatigue limit to tensile strength ratio.

This is probably because moving dislocations introduced upon steel plate production serve as a dislocation hardening factor and contribute to higher static strength, but cause cyclic softening during repeated deformation, namely, during a fatigue test, and thereby less contribute to higher fatigue strength. In particular, a steel plate having a dislocation density ρ of greater than 2.5× 10¹⁵ m⁻¹ as determined by X-ray diffractometry (XRD) undergoes significant improvement in static strength due to dislocation hardening and tends to have a lower fatigue limit to tensile strength ratio. The dislocation density ρ is preferably 2.0× 10¹⁵ m⁻¹ or less, and more preferably 1.5× 10¹⁵ m⁻¹ or less. The dislocation density ρ is 5.0× 10¹³ m⁻¹ or more in terms of lower limit.

Fig. 1 depicts schematic explanatory views of a steel plate according to the present invention. Specifically, Figs. 1(a) and 1(b) are a schematic perspective view and a schematic side view, respectively, of the steel plate according to the present invention. Figs. 1(a) and 1(b) illustrates a rolling direction L, a transverse direction (width direction) W, a thickness direction D, a steel plate surface S1, and a section S2 in the thickness direction D in parallel with the rolling direction L.

The inventors made investigations on various steel plates having different chemical compositions and different microstructure morphologies to examine fatigue properties. As a result, the inventors found that a steel plate is allowed to have excellent fatigue properties by controlling the microstructure of a longitudinal section (namely, the section S2 in Figs. 1(a) and 1(b)) as follows, where the longitudinal section is in parallel with the rolling direction, and where the microstructure is in a surface layer at a position adjacent to the steel plate surface S1, for example, in a surface layer at a position about 1 to about 3 mm deep from the steel plate surface S1 in the thickness direction. The surface layer herein is defined to be at a portion about 1 to about 3 mm deep from the steel plate surface, in order to evaluate a surface layer of the steel plate itself excluding a scale layer, because the steel plate surface immediately after production may include the scale layer of about 0.1 to about 2 mm depth (thickness) when produced under some production conditions.

The ferrite and upper bainite are phases that are relatively resistant to introduction of moving dislocations upon formation of the phases, as compared with other phases. This restrains the fatigue limit to tensile strength ratio from decreasing and contributes to longer life leading to crack initiation. To offer these advantageous effects, the microstructure in the surface layer is controlled to include at least one of ferrite and upper bainite in a total fraction of 80 area percent or more. The fraction of the at least one of ferrite and upper bainite is preferably 85 area percent or more, and more preferably 90 area percent or more. In terms of upper limit, the fraction of the at least one of ferrite and upper bainite is 100 area percent, but is typically about 98 area percent or less.

The grains of ferrite and upper bainite in the surface layer, if coarsen, may often undergo stress concentration, which causes cracks. When cracks after crack initiation collide with grains, the cracks stop and bypass the grains, and this restrains crack propagation. However, if the grains are coarse, cracks collide with the grains in a relatively smaller frequency. Thus, it is considered that the fatigue crack propagation in the surface layer is not sufficiently restrained. Based on these findings and considerations, the effective grain size of grains is specified to be 10.0 µm or less, where the grains herein are each defined as a region surrounded by high-angle grain boundaries with a misorientation of 15° or more between adjacent grains of ferrite or upper bainite. The term "effective grain size" refers to an average length of the grains in the thickness direction.

The effective grain size of the grains of at least one of ferrite and upper bainite is preferably 6 pm or less, and more preferably 5 pm or less. The lower limit of the effective grain size of the grains of at least one of ferrite and upper bainite is typically greater than about 2 pm.

The upper bainite phase can have a smaller size as compared with the ferrite phase, but is attended with shear deformation upon transformation, to which moving dislocations are readily introduced In particular, bainitic transformation, when allowed to occur at a low temperature, often gives a lower bainite phase containing a large amount of moving dislocations. To restrain the lower bainite phase from forming, the bainite transformation start temperature Bs is preferably controlled appropriately. From this viewpoint, the bainite transformation start temperature Bs calculated according to Expression (1) is preferably 640°C or higher, and more preferably 660°C or higher.

The remainder microstructure excluding the ferrite and the upper bainite in the surface layer is controlled to have an average equivalent circle diameter of 3.0 µm or less. The remainder microstructure is controlled to have an average equivalent circle diameter of 3.0 pm or less, because the remainder microstructure, if having an average equivalent circle diameter greater than 3.0 pm, may cause toughness and other properties to significantly deteriorate. The average equivalent circle diameter of the remainder microstructure is preferably 2.5 µm or less, and more preferably 2.0 pm or less in terms of upper limit; and is 0.5 pm or more in terms of lower limit. The remainder microstructure excluding the ferrite and the upper bainite in the surface layer basically includes martensite, martensite-austenite constituent (MA), pearlite, and pseudo-pearlite.

Among them, the martensite-austenite constituent, which is formed typically in cooling process after rolling, undergoes expansive transformation in its formation process, introduces moving dislocations into the matrix, and causes the steel plate to have a shorter life leading to crack initiation. To eliminate or minimize this, the proportion of the martensite-austenite constituent in the remainder microstructure in the surface layer is controlled to be an area percent of 5% or less. The area percent of the martensite-austenite constituent is preferably minimized, and is more preferably 3% or less, furthermore preferably 1% or less, and most preferably 0%.

Next, such a chemical composition of the steel plate according to the present invention as to have better fatigue properties will be described. The steel plate according to the present invention, as being incorporated with C, Mn, Nb, and other alloy elements as appropriate, is allowed to surely have a fine ferrite phase and/or an upper bainite phase. Simultaneously, the steel plate, as being: controlled in elements to be added such as Si and Cu as appropriate, restrains dislocations from forming a cell structure, which causes fatigue crack initiation. Thus, the steel plate can have excellent fatigue properties. From these viewpoints, the elements are controlled in the following manner.

### C: 0.02 to 0.10 mass percent

Carbon (C) is important to allow the steel plate to have strength at certain level. To this end, the carbon content is specified to be 0.02 mass percent or more. The carbon content is preferably 0.03 mass percent or more, and more preferably 0.04 mass percent or more. In contrast, the steel plate, if containing carbon in an excessively high content, may have excessively high strength to fail to have desired tensile strength. In addition, this steel plate, when undergoing accelerated cooling, may have excessive hardenability, have a large dislocation density p, and offer lower fatigue properties. To eliminate or minimize these, the carbon content is controlled to be 0.10 mass percent or less, and is preferably 0.08 mass percent or less, and more preferably 0.06 mass percent or less.

### Mn: 1.0 to 2.0 mass percent

Manganese (Mn) has a significance to ensure hardenability so as to give a fine microstructure. To effectively offer this activity, the Mn content is specified to be 1.0 mass percent or more. The Mn content is preferably 1.2 mass percent or more, and more preferably 1.4 mass percent or more. However, the steel plate, if containing Mn in an excessively high content, may have excessive hardenability, have a higher dislocation density p, and fail to have sufficient fatigue properties. To eliminate or minimize these, the Mn content is controlled to be 2.0 mass percent or less, and is preferably 1.8 mass percent or less, and more preferably 1.6 mass percent or less.

### Nb: greater than 0 mass percent to 0.05 mass percent

Niobium (Nb) is effective for better hardenability and for a finer microstructure. To effectively offer these activities, the Nb content is preferably controlled to be 0.01 mass percent or more, and more preferably 0.02 mass percent or more. However, the steel plate, if containing Nb in an excessively high content, may have excessive hardenability and fail to have desired fatigue properties. To eliminate or minimize this, the Nb content is controlled to be 0.05 mass percent or less, and is preferably 0.04 mass percent or less, and more preferably 0.03 mass percent or less.

### Ti: greater than 0 mass percent to 0.05 mass percent

Titanium (Ti) effectively contributes to better hardenability and, simultaneously, forms TiN to allow the heat-affected zone upon welding to have a finer microstructure and to restrain reduction in toughness. To offer these activities, the Ti content is preferably 0.01 mass percent or more, and more preferably 0.02 mass percent or more. However, Ti, if contained in an excessively high content, may form coarse TiN particles and may cause the steel plate to have properties such as toughness at lower levels. To eliminate or minimize this, the Ti content is controlled to be 0.05 mass percent or less, and is preferably 0.04 mass percent or less, and more preferably 0.03 mass percent or less.

### Al: 0.01 to 0.06 mass percent

Aluminum (Al) is useful for deoxidation and, if contained in a content less than 0.01 mass percent, may fail to offer effective deoxidation. The Al content is preferably 0.02 mass percent or more, and more preferably 0.03 mass percent or more. However, the steel plate, if containing Al in an excessively high content, may have excessive hardenability, have a higher dislocation density p, and fail to offer desired fatigue properties. To eliminate or minimize these, the Al content is controlled to be 0.06 mass percent or less, and is preferably 0.05 mass percent or less, and more preferably 0.04 mass percent or less.

### Optionally Si in a content of 0.1 to 0.6 mass percent

Silicon (Si) contributes to solid-solution strengthening to a large extent and is necessary for ensuring the strength of the base metal Simultaneously, this element restrains the movements of dislocations and restrains the cell structure formation. To effectively offer these activities, the Si content is specified to be 0.1 mass percent or more. The Si content is preferably 0.2 mass percent or more, and more preferably 0.3 mass percent or more. However, the steel plate, if containing Si in an excessively high content, may include the remainder microstructure formed in excess and coarsely and may suffer from reduction in other properties such as toughness. To eliminate or minimize this, the Si content is controlled to be 0.6 mass percent or less, and is preferably 0.55 mass percent or less, and more preferably 0.5 mass percent or less.

### Cu: 0.1 to 0.6 mass percent

Copper (Cu) restrains the cross slip of dislocations and effectively restrains the cell structure formation. To effectively offer the activities, the Cu content is specified to be 0.1 mass percent or more. The Cu content is preferably 0.2 mass percent or more, and more preferably 0.3 mass percent or more. However, the steel plate, if containing Cu in an excessively high content, may not only have excessive hardenability, but also become susceptible typically to cracking upon hot working. To eliminate or minimize these, the Cu content is controlled to be 0.6 mass percent or less, and is preferably 0.55 mass percent or less, and more preferably 0.5 mass percent or less.

Si and Cu can offer the common activity of restraining cell structure formation of dislocations. From this viewpoint, the steel plate may contain these elements in combination. The effect of restraining cell structure formation of dislocations by Si and Cu is effectively offered when the total content of Si and Cu ([Si] + [Cu]) is 0.3 mass percent or more. The total content is preferably 0.4 mass percent or more. A preferred upper limit of the total content ([Si] + [Cu]) is the total of the preferred upper limits of the two elements.

### Ni: greater than 0 mass percent to 0.6 mass percent

Nickel (Ni) effectively contributes to better hardenability and contributes to a finer microstructure. Simultaneously, this element effectively restrains cracking upon hot working, where the cracking may more readily occur by the addition of Cu. To effectively offer these effects, Ni is preferably contained in a content of 0.1 mass percent or more, and more preferably 0.2 mass percent or more. However, the steel plate, if containing Ni in an excessively high content, may have excessive hardenability, have an excessively high dislocation density p, and thereby fail to have desired fatigue properties. To eliminate or minimize these, the Ni content is controlled to be 0.6 mass percent or less, more preferably 0.5 mass percent or less, and furthermore preferably 0.4 mass percent or less.

The steel plate, if having an excessively high Ni content [Ni] with respect to the Cu content [Cu], may hardly enjoy the effect of restraining cell structure formation of dislocations by Cu. To eliminate or minimize this, the ratio ([Ni]/[Cu]) of the Ni content [Ni] to the Cu content [Cu] is controlled to be less than 1.2, and more preferably 1.1 or less. The ratio ([Ni]/[Cu]) is 0.5 or more in terms of lower limit.

The steel plate according to the present invention includes the elements as mentioned above as a basic composition, with the remainder consisting of approximately iron. However, it is naturally accepted that inevitable impurities such as P, S, and N are contained in the steel The inevitable impurities are brought into the steel in circumstances of raw materials, facility materials, and production equipment. It is also effective that the steel plate according to the present invention positively contains one or more of elements below. The steel plate can have a still better property or properties according to the type(s) of elements) to be contained.

At least one element selected from the group consisting of V in a content of greater than 0 mass percent to 0.5 mass percent, Cr in a content of greater than 0 mass percent to 1.0 mass percent or less, and Mo in a content of greater than 0 mass percent to 0.5 mass percent

Vanadium (V), chromium (Cr), and molybdenum (Mo) effectively allow the steel plate to have better hardenability and to have a finer microstructure. To offer these activities, the steel plate preferably contains each of V in a content of 0.01 mass percent or more, Cr in a content of 0.1 mass percent or more, and Mo in a content of 0.01 mass percent or more alone or in combination. However, the steel plate, if containing at least one of these elements in an excessively high content, may have excessive hardenability, have an excessively high dislocation density p, and fail to have desired fatigue properties. To eliminate or minimize these, the contents of V, Cr, and Mo are preferably controlled to be respectively 0.5 mass percent or less, 1.0 mass percent or less, and 0.5 mass percent or less. The contents of V, Cr, and Mo are more preferably controlled to be respectively 0.4 mass percent or less, 0.8 mass percent or less, and 0.4 mass percent or less.

### B: greater than 0 mass percent to 0.005 mass percent

Boron (B) contributes to better hardenability and, in particular, restrains a coarse ferrite phase from forming, and thereby allows a fine upper bainite phase to form more readily. To offer these effects, the boron content is preferably controlled to be 0.0005 mass percent or more, and more preferably 0.001 mass percent or more. However, the steel plate, if containing boron in an excessively high content, may have excessive hardenability, have an excessively high dislocation density p, and fail to have desired fatigue properties. To eliminate or minimize these, the boron content is preferably controlled to be 0.005 mass percent or less, and more preferably 0.004 mass percent or less.

The thickness of the steel plate according to the present invention is not limited, but having an excessively small thickness, may less offer longer crack propagation life. From this viewpoint, the steel plate has a thickness of preferably 6 mm or more, and more preferably 10 mm or more.

The steel plate according to the present invention meets the conditions (requirements) and is not limited in production method. However, it is preferred to control production conditions as mentioned below, so as to give the microstructure morphology for better fatigue properties. The production conditions are conditions in a series of production process for the steel plate using a slab, such as a slab, having a chemical composition within the ranges. In the production process, a steel is made via ingot making and casting, and is subjected to hot rolling. Specifically, the production conditions include the heating temperature before hot rolling; the cumulative compression reduction in the entire hot rolling process; the finish-rolling temperature; the average cooling rate from the finish-rolling temperature or 800°C, whichever is lower, down to 600°C; and the cooling stop temperature.
Temperature of heating before hot rolling: 1000°C to 1200°C
Cumulative compression reduction in entire hot rolling process: 70% or more
Finish-rolling temperature: from the Ar₃ transformation temperature to (the Ar₃ transformation temperature + 150°C)
Average cooling rate from the finish-rolling temperature or 800°C, whichever is lower, down to 600°C: 15°C/second or less
Cooling stop temperature: 500°C or higher

Before the hot rolling, the slab is preferably heated up to a temperature range of 1000°C to 1200°C, and more preferably up to 1050°C or higher. The heating is preferably performed up to a temperature range of 1000°C or higher so as to eliminate or minimize coarsening of grains and to still ensure a cumulative compression reduction in hot rolling of 70% or more, as mentioned below. However, the heating, if performed up to an excessively high temperature of higher than 1200°C, may fail to contribute to refinement (size reduction) of the microstructure even when sufficient compression reduction is applied. To eliminate or minimize this, the heating temperature is preferably controlled to be 1200°C or lower, and more preferably 1150°C or lower.

The cumulative compression reduction in the entire hot rolling process is preferably 70% or more, and more preferably 75% or more. To reduce the microstructure size, in particular to reduce the effective grain size, sufficient compression reduction is to be applied in the non-recrystallization temperature range.

In addition, the finish-rolling temperature is preferably controlled within the range of the Ar₃ transformation temperature to the (Ar₃ transformation temperature + 150°C) so as to ensure desired fine microstructure and to still restrain excessive dislocations from being introduced into the microstructure after rolling (as-rolled microstructure). The finish-rolling temperature is more preferably controlled within the range of (the Ar₃ transformation temperature + 20°C) to (the Ar₃ transformation temperature + 100°C).

The "cumulative compression reduction" is a value calculated according to Expression (4): $Cumulative compression reduction = \left({t}_{0}-{t}_{1}\right) / {t}_{2} \times 100$ where to represents the slab rolling start thickness (in millimeter (mm)) when the temperature at a position 3 mm deep from the surface falls within the rolling temperature range; t₁ represents the rolling finish thickness of the slab (in mm) when the temperature at a position 3 mm deep from the surface falls within the rolling temperature range; and t₂ represents the thickness of the slab, such as a slab, before the rolling.

The Ar₃ transformation temperature employed herein is a value determined according to Expression (5): ${Ar}_{3} transformation temperature = 910 - 230 \left[C\right] + 25 \left[Si\right] - 74 \left[Mn\right] - 56 \left[Cu\right] - 16 \left[Ni\right] - 9 \left[Cr\right] - 5 \left[Mo\right] - 1620 \left[Nb\right]$ where [C], [Si], [Mn], [Cu], [Ni], [Cr], [Mo], and [Nb] represent contents (in mass percent) respectively of C, Si, Mn, Cu, Ni, Cr, Mo, and Nb.

After hot rolling finish, cooling is preferably performed at an average cooling rate of 15°C/second or less from the finish-rolling temperature or 800°C, whichever is lower, down to 600°C or lower. The cooling, if performed at an average cooling rate greater than 15°C/second, may cause the microstructure transformation to complete at an approximately low temperature unless a process such as isothermal holding is performed. This causes excessive introduction of dislocations and fails to give desired fatigue properties. The average cooling rate is more preferably 10°C/second or less.

The cooling at the average cooling rate may be stopped at a temperature (namely, cooling stop temperature) of 500°C or higher. This restrains coarse ferrite phase formation and ensures a fine ferrite or upper bainite phase. The cooling, if stopped at a temperature lower than 500°C, may cause the transformation to complete at a low temperature, cause excessive dislocations to be introduced, and fail to give desired fatigue properties.

The temperature range within which cooling is performed at the average cooling rate is from 800°C down to 600°C when the finish-rolling temperature is higher than 800°C; and is from the finish-rolling temperature down to 600°C when the finish-rolling temperature is lower than 800°C. The average cooling rate in terms of lower limit is preferably 3.0°C/second or more, from the viewpoint of microstructure control in the steel plate.

### Examples

The present invention will be illustrated in further detail with reference to several examples (experimental examples) below. It should be noted, however, that the examples are by no means intended to limit the scope of the invention; that various changes and modifications can naturally be made therein without deviating from the scope of the invention as described herein; and all such changes and modifications should be considered to be within the scope of the invention.

### Experimental Example 1

Ingots of steels having chemical compositions corresponding to Steels A to W as given in Table 1 were made via melting and casting according to a common ingot-making technique, subjected to hot rolling under conditions of rolling condition types "a" to "l" given in Table 2, and yielded steel plates having a thickness of 20 mm. In Table 1, an element indicated with "-" was not added; and the symbol "[Si]+[Cu] "refers to the total content of Si and Cu. The Ar₃ transformation temperatures given in Table 1 are values determined according to Expression (5). In Table 2, the term "entire hot rolling process cumulative compression reduction" refers to the cumulative compression reduction in the entire hot rolling process.

**[Table 1]**

| Steel | Chemical | composition | | (in | mass percent) | | with | the remainder | consisting | of | iron and | inevitable | impurities | Bs | [Si]+[Cu] | [Ni]/[Cu] | Ar₃ transformation temperature | Left-side value of Expression (2) | Left-side value of Expression (3) |
|---|---|---|---|---|---|---|---|---|---|---|---|---|---|---|---|---|---|---|---|
| | C | Si | Mn | Al | Cu | Ni | Cr | Mo | V | Nb | Ti | B | N | | | | | | |
| A | 0.05 | 0.31 | 1.56 | 0.03 | 0.31 | 0.30 | - | - | - | 0.019 | 0.015 | 0.0012 | 0.0044 | 665 | 0.62 | 0.97 | 738 | 49 | 0.00 |
| C | 0.06 | 0.25 | 1.59 | 0.03 | 0.33 | 0.16 | - | - | - | 0.020 | 0.015 | 0.0009 | 0.0040 | 665 | 0.58 | 0.48 | 731 | 45 | 0.03 |
| D | 0.05 | - | 1.55 | 0.03 | 0.54 | 0.51 | - | - | - | 0.019 | 0.013 | 0.0010 | 0.0052 | 658 | 0.54 | 0.94 | 715 | 45 | 0.00 |
| E | 0.05 | 0.38 | 1.81 | 0.04 | 0.24 | 0.20 | - | - | - | 0.018 | 0.021 | 0.0009 | 0.0048 | 646 | 0.62 | 0.83 | 728 | 53 | 0.10 |
| G | 0.07 | 0.44 | 1.55 | 0.03 | 0.33 | 0.29 | - | - | - | 0.025 | 0.016 | - | 0.0043 | 661 | 0.77 | 0.88 | 727 | 54 | 0.03 |
| H | 0.04 | 0.42 | 1.55 | 0.03 | 0.32 | 0.32 | 0.2 | - | - | 0.019 | 0.018 | 0.0015 | 0.0047 | 654 | 0.74 | 1.00 | 741 | 53 | 3.84 |
| I | 0.04 | 0.41 | 1.57 | 0.03 | 0.32 | 0.31 | - | 0.02 | - | 0.023 | 0.019 | 0.0009 | 0.0047 | 665 | 0.73 | 0.97 | 735 | 53 | 0.26 |
| J | 0.05 | 0.39 | 1.52 | 0.03 | 0.35 | 0.30 | - | - | 0.02 | 0.023 | 0.017 | 0.0008 | 0.0042 | 669 | 0.74 | 0.86 | 734 | 52 | 0.06 |
| K | 0.01 | 0.41 | 1.55 | 0.03 | 0.31 | 0.25 | - | - | - | 0.019 | 0.016 | 0.0009 | 0.0043 | 679 | 0.72 | 0.81 | 751 | 51 | 0.03 |
| L | 0.15 | 0.42 | 1.55 | 0.03 | 0.32 | 0.18 | - | - | - | 0.020 | 0.016 | 0.0007 | 0.0043 | 643 | 0.74 | 0.56 | 718 | 51 | 0.03 |
| M | 0.05 | 0.10 | 1.61 | 0.03 | - | - | - | - | - | 0.021 | 0.018 | 0.0013 | 0.0044 | 672 | 0.10 | - | 748 | 32 | 0.06 |
| N | 0.05 | 1.00 | 1.55 | 0.03 | 0.31 | 0.23 | - | - | - | 0.020 | 0.017 | 0.0014 | 0.0042 | 668 | 1.31 | 0.74 | 755 | 72 | 0.06 |
| 0 | 0.03 | 0.34 | 2.12 | 0.03 | 0.29 | 0.18 | - | - | - | 0.022 | 0.017 | 0.0013 | 0.0049 | 624 | 0.63 | 0.62 | 700 | 58 | 0.01 |
| P | 0.05 | 0.35 | 0.55 | 0.03 | 0.33 | 0.32 | - | - | - | 0.020 | 0.019 | 0.0013 | 0.0052 | 755 | 0.68 | 0.97 | 811 | 33 | 0.03 |
| Q | 0.05 | 0.52 | 1.57 | 0.03 | 1.50 | - | - | - | - | 0.018 | 0.016 | 0.0012 | 0.0045 | 675 | 2.02 | 0.00 | 682 | 70 | 0.01 |
| R | 0.03 | 0.21 | 1.51 | 0.03 | 0.25 | 1.20 | - | - | - | 0.019 | 0.019 | 0.0010 | 0.0051 | 642 | 0.46 | 4.80 | 733 | 59 | 0.03 |
| S | 0.06 | 0.41 | 1.56 | 0.03 | 0.30 | 0.15 | 1.5 | - | - | 0.020 | 0.020 | 0.0008 | 0.0045 | 563 | 0.71 | 0.50 | 726 | 50 | 28.60 |
| T | 0.04 | 0.42 | 1.52 | 0.03 | 0.29 | 0.28 | - | 1.00 | - | 0.021 | 0.018 | 0.0009 | 0.0045 | 589 | 0.71 | 0.97 | 739 | 51 | 10.06 |
| U | 0.03 | 0.41 | 1.55 | 0.03 | 0.31 | 0.22 | - | - | 1.00 | 0.025 | 0.018 | 0.0009 | 0.0044 | 674 | 0.72 | 0.71 | 737 | 51 | 0.06 |
| V | 0.08 | 0.39 | 1.82 | 0.03 | 0.31 | 0.19 | 0.8 | 0.30 | - | 0.022 | 0.019 | 0.0008 | 0.0046 | 557 | 0.70 | 0.61 | 702 | 55 | 18.27 |
| W | 0.05 | 0.15 | 1.10 | 10.03 | 0.16 | 0.05 | - | - | - | 0.019 | 0.015 | 0.0012 | 0.0044 | 665 | 0.31 | 0.97 | 738 | 28 | 0.00 |

**[Table 2]**

| Rolling condition type | Heating temperature (°C) | Cumulative compression reduction in entire hot rolling process (%) | Cumulative compression reduction in non-recrystallization range (%) | Finish-rolling temperature (°C) | Average cooling rate down to 600°C (°C/sec) | Cooling stop temperature (°C) |
|---|---|---|---|---|---|---|
| a | 1150 | 90 | 75 | 820 | 5 | 583 |
| b | 1150 | 85 | 75 | 800 | 12 | 580 |
| c | 1100 | 80 | 75 | 820 | AC* | 570 |
| d | 1175 | 80 | 75 | 870 | 3.1 | 600 |
| e | 1150 | 75 | 75 | 750 | 8.1 | 580 |
| f | 1150 | 80 | 75 | 820 | 5.1 | 520 |
| g | 1250 | 90 | 75 | 820 | 5 | 580 |
| h | 1150 | 50 | 75 | 820 | 5 | 580 |
| i | 1150 | 90 | 75 | 700 | 5 | 580 |
| j | 1150 | 90 | 75 | 820 | 30 | 580 |
| k | 1150 | 90 | 75 | 800 | 5 | 150 |
| l | 1150 | 90 | 95 | 820 | 5 | 580 |

| | | | | | | |
|---|---|---|---|---|---|---|
| * AC: air cooling at an average cooling rate of 0.8°C/sec | | | | | | |

The steel plates were each subjected to measurements of the microstructure and effective grain size of the steel plate, the size of the remainder microstructure as a second phase, the tensile strength, the fatigue properties, and the dislocation density p, according to procedures as follows. Test specimens in all the measurements were sampled so that the measurement position be a position 3 mm deep from the steel plate surface.

### Steel Plate Surface Layer Microstructure

A sample was cut out at a position 3 mm deep from the steel plate surface so as to expose a plane in parallel with the rolling direction of the steel plate and in perpendicular to the steel plate surface. This was polished using wet emery papers of #150 to #1000 and was then polished to a mirror-smooth state using a diamond abrasive as an abrasive. The mirror-smooth test specimen was etched with 2% nitric acid-ethanol solution, i.e., Nital solution, the etched test specimen was observed in three view fields in an observation area of 3.71× 10⁻² mm² at 400-fold magnification, images of which were taken and analyzed using an image analyzing software Image Pro Plus ver. 4.0 supplied by Media Cybernetics so as to fractionate phases in the microstructure. Values in the three view fields were averaged, and the average was defined as the area percentages of the individual phases. The observation area was such that one view field in a size of 166 µm in the thickness direction and 222.74 pm in the rolling direction was defined around the position 3 mm deep from the steel plate surface.

### Ferrite and Upper Bainite Effective Grain Sizes in Surface Layer

The effective grain size of ferrite and/or upper bainite was analyzed at a position 3 mm deep from the steel plate surface in a longitudinal section in parallel with the rolling direction of the steel plate. The measurement was performed by scanning electron microscope (SEM)-electron backscatter pattern analysis (EBSP). Specifically, a grain size was measured, where the "grain" is defined as a region surrounded by a high-angle grain boundary having a misorientation between adjacent grains of 15° or more. The measurement was performed using an EBSP system (trade name OIM) supplied by TEX SEM Laboratories in combination with a SEM, in a measurement area of 200 µm by 200 pm at a measurement step (interval) of 0.5 pm. A measurement point having a confidence index of less than 0.1 was excluded from the analysis object, where the confidence index indicates the reliability of a measurement orientation. The cut lengths of the grain boundaries thus determined were measured at 100 points in the thickness direction, and an average of the cut lengths was defined as the effective grain size. However, a measurement with an effective grain size of 2.0 µm or less was determined as a measurement noise and excluded. The observation area was determined as a region around the position 3 mm deep from the steel plate surface with a spread of 100 pm on both sides in the thickness direction.

### Remainder Microstructure Size

The size of the remainder microstructure excluding the ferrite and the upper bainite was determined in the following manner. A sample was cut out at a position 3 mm deep from the steel plate surface so as to expose a plane in parallel with the rolling direction of the steel plate and in perpendicular to the steel plate surface. This was polished using wet emery papers of #150 to #1000 and was then polished to a mirror-smooth state using a diamond abrasive as an abrasive. The mirror-smooth test specimen was etched with 2% nitric acid-ethanol solution, i.e., Nital solution, the etched test specimen was observed in an observation area of 3.71× 10⁻² mm² at 400-fold magnification. The observation area was determined as a region around the position 3 mm deep from the steel plate surface with a spread of 100 pm on both sides in the thickness direction. Images of the observed test specimen were taken and analyzed using the image analyzing software, an area per one grain of the remainder microstructure was calculated, and the equivalent circle diameter of grains of the remainder microstructure was determined from the calculated area. In this experimental example, measurements in three view fields were averaged, and the average was defined as the equivalent circle diameter.

Of the remainder microstructure, the area percentage of MA was determined in the following manner. The mirror-smooth test specimen after polishing to a mirror-smooth state was etched with a LePera etchant and observed in an observation area of 3.71× 10⁻² mm² at 400-fold magnification. A phase corroded to white was defined as the MA, images of which were taken and analyzed using the image analyzing software to fractionate phases. Measurements in five view fields were averaged, and the average was defined as the area percentage of MA. The LePera etchant was a 5:6:1 mixture of a solution A, a solution B, and ethanol The solution A was a solution of 3 g of picric acid in 100 ml of ethanol. The solution B was a solution of 1 g of sodium disulfite in 100 ml of distilled water.

### Tensile Strength

The tensile strength TS was measured by sampling a tensile test specimen having a thickness of 4 mm and a gauge length of 35 mm from each steel plate at a position 2 to 6 mm deep from the steel plate surface, and subjecting the test specimen to a tensile test according to JIS Z 2241:2011.

### Fatigue Properties

The fatigue properties were determined in the following manner. A steel plate sample having a thickness of 4 mm was cut out from each steel plate at a position 2 to 6 mm deep from the steel plate surface, from which a test specimen as illustrated in Fig. 2 was prepared. The test specimen surface was polished with emery papers up to #1200 to eliminate or minimize influence of surface conditions. The resulting test specimen was subjected to a fatigue test using a servo-electric hydraulic fatigue tester supplied by INSTRON Co., Ltd. under conditions as follows.
Testing environment: room temperature, in the air
Control type: load control
Control waveform: sinusoidal wave
Stress ratio R: -1
Testing frequency: 20 Hz
Number of cycles to complete testing: 5000000

The fatigue properties are affected by the tensile strength TS. To eliminate or minimize the influence of the tensile strength, a 5000000-cycle fatigue limit to tensile strength ratio was determined, and a sample, when having a 5000000-cycle fatigue limit to tensile strength ratio of greater than 0.51, was accepted herein. The 5000000-cycle fatigue limit to tensile strength ratio is a value determined by dividing a 5000000-cycle fatigue limit by the tensile strength TS. The 5000000-cycle fatigue limit was determined in the following manner. Each test specimen was subjected to a fatigue test at such a stress amplitude as to give a stress amplitude σa to tensile strength TS ratio (σa/TS) of 0.51, and whether the test specimen underwent rupture upon the 5000000th cycles was examined.

### Dislocation Density ρ

The dislocation density ρ was determined by subjecting each sample to X-ray diffractometry to determine a half peak width (full-width at half maximum) of α-Fe, and calculating the dislocation density from the half peak width. The measurement conditions and principle will be illustrated below. An analyzer used herein was an X-ray diffractometer RAD-RU300 (trade name, supplied by Rigaku Corporation), with a cobalt tube as a target. The half peak width was calculated from the results of X-ray diffractometry via peak fitting, based on which the dislocation density ρ was calculated according to Expression (6): $ρ \left({m}^{- 1}\right) = - 14.4 {ε}^{2} / {b}^{2}$ where ε represents the strain; and b represents the Burgers vector (=0.25×10⁻⁹ m).

The strain ε is a value calculated according to the Hall method based on Expression (7) and Expression (8): $β cos θ / λ = 0.9 / D + 2 ε sin θ / λ$ ${β}^{2} = {{β}_{m}}^{2} - {{β}_{s}}^{2}$ where β represents the true half peak width (in radian (rad)); θ represents the Bragg angle (in degree (°)); λ represents the wavelength (in nanometer (nm)) of incident X ray; D represents the crystal size (in nm); βₘ represents the measured half peak width; and βₛ represents the half peak width (apparatus constant) of a sample with no strain. The true half peak width β was calculated from βₘ and βₛ according to Expression (8), and this was substituted into Expression (7), based on which βoos θ/λ - sin θ/λ was plotted. Three points, i.e., (110), (211), and (220) points were fitted by the method of least squares. The strain ε was calculated from the slope (2ε) of the fitting line and was substituted into Expression (6) to calculate the dislocation density ρ.

Table 3 presents, of each steel plate, the microstructure, the effective grain size, the remainder microstructure size, the tensile strength TS, the fatigue properties, and the dislocation density ρ.

**[Table 3]**

| Test number ' | Steel | Rolling condition type | Tensile strength TS (MPa) | Microstructure* of steel plate surface layer | Total of ferrite and upper bainite in steel plate surface layer (area percent) | Effective grain size (µm) | Remainder microstructure size (µm) | MA fraction in steel plate surface layer (area percent) | *ρ* [×10¹³m⁻¹] | Fatigue properties |
|---|---|---|---|---|---|---|---|---|---|---|
| 1 | A | a | 581 | F+B | 95 | 5.5 | 1.1 | 1.1 | 1.2 | no rupture |
| 3 | C | a | 529 | F+B | 94 | 4.9 | 0.8 | 0.7 | 1.3 | no rupture |
| 4 | D | a | 630 | F+B | 93 | 4.6 | 0.9 | 0.1 | 1.7 | no rupture |
| 5 | E | a | 559 | F+B | 92 | 6.2 | 1.0 | 0.5 | 0.9 | no rupture |
| 7 | G | a | 536 | F+B | 94 | 5.7 | 1.4 | 0.7 | 0.8 | no rupture |
| 8 | H | a | 610 | F+B | 90 | 4.4 | 0.9 | 0.6 | 1.7 | no rupture |
| 9 | I | a | 621 | F+B | 92 | 4.3 | 0.8 | 0.2 | 1.6 | no rupture |
| 10 | J | a | 617 | F+B | 95 | 4.5 | 1.0 | 0.3 | 1.6 | no rupture |
| 11 | A | b | 627 | F+B | 91 | 4.3 | 0.7 | 1.1 | 1.7 | no rupture |
| 12 | A | c | 555 | F | 96 | 6.1 | 1.6 | 01 | 0.8 | no rupture |
| 13 | A | d | 571 | F+B | 96 | 5.6 | 0.7 | 1.8 | 1.2 | no rupture |
| 14 | A | e | 589 | F+B | 92 | 5.8 | 1.1 | 1.2 | 1.0 | no rupture |
| 15 | A | f | 629 | F+B | 93 | 4.5 | 0.9 | 0.4 | 1.8 | no rupture |
| 16 | A | l | 638 | F+B | 98 | 3.5 | 0.6 | 0.3 | 1.8 | no rupture |
| 17 | W | b | 621 | F+B | 90 | 4.4 | 1,2 | 0.4 | 1.2 | no rupture |
| 18 | K | c | 410 | F | 91 | - | - | 0.1 | - | - |
| 19 | L | a | 791 | B | 3B | - | - | 0,4 | - | - |
| 20 | M | a | 581 | F+B | 92 | 4.8 | 1.4 | 0.5 | 1.7 | rupture |
| 21 | N | a | 624 | F+B | 81 | 6.0 | 4.2 | 2.1 | 1.7 | rupture |
| 22 | O | a | 701 | B | 68 | 4.4 | 0.8 | 1.1 | 3.7 | rupture |
| 23 | P | a | 462 | F | 83 | 10.2 | 1.4 | 0.1 | 1.8 | rupture |
| 24 | Q | a | 616 | F+B | 83 | 6.2 | 1.0 | 1.3 | 5.0 | rupture |
| 25 | R | a | 631 | F+B | 87 | 5.8 | 1.1 | 1.4 | 4.6 | rupture |
| 26 | S | a | 647 | F+B | 85 | 4.5 | 0.8 | 1.1 | 3.8 | rupture |
| 27 | T | a | 638 | F+B | 84 | 4.7 | 0.8 | 1.0 | 3.7 | rupture |
| 28 | U | a | 625 | F+B | 85 | 5.3 | 1.1 | 1.1 | 4.4 | rupture |
| 29 | V | a | 625 | F+B | 84 | 5.0 | 1.0 | 0.9 | 3.8 | rupture |
| 30 | A | g | 587 | B | 91 | 10.2 | 0.9 | 5.3 | 1.1 | rupture |
| 31 | A | h | 591 | F+B | 90 | 10.3 | 0.3 | 0**.**2 | 1.1 | rupture |
| 32 | A | i | 612 | F | 83 | 5.3 | 1.3 | 0.3 | 2.9 | rupture |
| 33 | A | j | 659 | B | 96 | 4.9 | 0.8 | 1.5 | 3.1 | rupture |
| 34 | A | k | 643 | B | 95 | 5.1 | 0.7 | 0.2 | 2.7 | rupture |

| | | | | | | | | | | |
|---|---|---|---|---|---|---|---|---|---|---|
| * F represents ferrite, B represents bainite, and M represents martensite, where, when the microstructure is indicated as "B", the remainder microstructure is martensite. | | | | | | | | | | |

These results indicate as follows. Specifically, Test Nos.1 to 17 were produced under appropriately controlled conditions using steels having appropriately controlled chemical compositions, met the conditions in the surface layer specified in the present invention, and offered excellent fatigue properties.

In contrast, Test Nos.18 to 34 were samples failing to meet at least one of the conditions specified in the present invention, and each had poor fatigue properties. Among them, Test No. 18 employed a steel plate derived from Steel K having a low carbon content and failed to have a tensile strength TS at the predetermined level. Accordingly, other properties than the microstructure were not evaluated in this sample. Test No. 19 employed a steel plate derived from Steel L having an excessively high carbon content and had an excessively high tensile strength TS. Accordingly, other properties than the microstructure were not evaluated in this sample.

Test No. 20 employed a steel plate derived from Steel M not meeting the condition that "the total content of Si and Cu is 0.3% or more", failed to restrain cell structure formation of dislocations, and had inferior fatigue properties. Test No. 21 employed a steel plate derived from Steel N having an excessively high Si content, had an excessively large size of the remainder microstructure, and had inferior fatigue properties.

Test No. 22 employed a steel plate derived from Steel O having an excessively high Mn content, had a high tensile strength TS and a high dislocation density p, and offered inferior fatigue properties. Test No. 23 employed a steel plate derived from Steel P having an excessively low Mn content, failed to have a tensile strength TS at the predetermined level, had an excessively large effective grain size, and offered inferior fatigue properties.

Test No. 24 employed a steel plate derived from Steel Q having an excessively high Cu content, had an excessively high dislocation density p, and offered inferior fatigue properties. Test No. 25 employed a steel plate derived from Steel R having an excessively high Ni content and not meeting the condition: [Ni]/[Cu]<1.2. This sample had an excessively high dislocation density p, and offered inferior fatigue properties.

Test No. 26 employed a steel plate derived from Steel S having an excessively high Cr content, had an excessively high dislocation density p, and offered inferior fatigue properties. Test No. 27 employed a steel plate derived from Steel T having an excessively high Mo content, had an excessively high dislocation density p, and offered inferior fatigue properties.

Test No. 28 employed a steel plate derived from Steel U having an excessively high V content, had an excessively high dislocation density p, and offered inferior fatigue properties. Test No. 29 employed a steel plate derived from Steel V having a bainite transformation start temperature Bs lower than 640°C, had an excessively high dislocation density p, and offered inferior fatigue properties.

Test No. 30 was a sample produced via rolling under conditions of the type g with an excessively high heating temperature in hot rolling, had an excessively large effective grain size, and offered inferior fatigue properties. Test No. 31 was a sample produced via rolling under conditions of the type h with an excessively low cumulative compression reduction in hot rolling, had an excessively large effective grain size, and offered inferior fatigue properties.

Test No. 32 was a sample produced via rolling under conditions of the type i with an excessively low finish-rolling temperature, had an excessively high dislocation density p, and offered inferior fatigue properties. Test No. 33 was a sample produced via rolling under conditions of the type j with an excessively high average cooling rate down to 600°C, had an excessively high dislocation density p, and offered inferior fatigue properties. Test No. 34 was a sample produced via rolling under conditions of the type k with an excessively low cooling stop temperature, had an excessively high dislocation density p, and offered inferior fatigue properties.

## Claims

1. A steel plate comprising:
C in a content of 0.02 to 0.10 mass percent;
Mn in a content of 1.0 to 2.0 mass percent;
Nb in a content of greater than 0 mass percent to 0.05 mass percent;
Ti in a content of greater than 0 mass percent to 0.05 mass percent;
Al in a content of 0.01 to 0.06 mass percent;
Cu in a content of 0.1 to 0.6 mass percent; and
Ni in a content of greater than 0 mass percent to 0.6 mass percent, where a ratio [Ni]/[Cu] of the Ni content [Ni] to the Cu content [Cu] is 0.5 to less than 1.2;
optionally comprising Si in a content of 0.1 to 0.6 mass percent;
where a total content of Si and Cu is 0.3 mass percent or more,
optionally comprising, in chemical composition, at least one selected from the group consisting of:
(b) at least one element selected from the group consisting of:
V in a content of greater than 0 mass percent to 0.5 mass percent;
Cr in a content of greater than 0 mass percent to 1.0 mass percent or less; and
Mo in a content of greater than 0 mass percent to 0.5 mass percent; and
(c) B in a content of greater than 0 mass percent to 0.005 mass percent, with the remainder consisting of iron and inevitable impurities,
wherein a microstructure of a surface layer of the steel plate comprises at least one of ferrite and upper bainite in a total fraction of 80 area percent to 100 area percent as determined with the measurement method defined in the description under the heading "Steel Plate Surface Layer Microstructure",
wherein, of the microstructure of the surface layer, the remainder microstructure excluding the ferrite and the upper bainite optionally has a fraction of martensite-austenite constituent of 0 area percent to 5 area percent as determined with the measurement method defined in the description under the heading "Remainder Microstructure Size",
wherein grains of the at least one of ferrite and upper bainite have an effective grain size of 2 µm to 10.0 µm, wherein the effective grain size refers to an average length of the grains in the thickness direction as determined with the measurement method defined in the description under the heading "Ferrite and
Upper Bainite Effective Grain Sizes in Surface Layer", wherein, of the microstructure of the surface layer, grains of a remainder microstructure excluding the ferrite and the upper bainite have an average equivalent circle diameter of 0.5 µm to 3.0 µm as determined with the measurement method defined in the description under the heading "Remainder Microstructure Size", and
wherein the steel plate has a dislocation density ρ of 5.0× 10¹³ m⁻¹ to 2.5× 10¹⁵ m⁻¹ as determined by X-ray diffractometry with the measurement method defined in the description under the heading "Dislocation Density p".

2. The steel plate according to claim 1,
wherein the steel plate has a bainite transformation start temperature Bs of 640°C or higher, where the bainite transformation start temperature is calculated from the chemical composition according to Expression (1): $Bs \left(°C\right) = 830 - 270 \left[C\right] - 90 \left[Mn\right] - 37 \left[Ni\right] - 70 \left[Cr\right] - 83 \left[Mo\right]$ wherein [C], [Mn], [Ni], [Cr], and [Mo] represent contents (in mass percent) respectively of C, Mn, Ni, Cr, and Mo.

## Patentansprüche

1. Stahlplatte, umfassend:
C in einem Gehalt von 0,02 bis 0,10 Massenprozent;
Mn in einem Gehalt von 1,0 bis 2,0 Massenprozent;
Nb in einem Gehalt von mehr als 0 Massenprozent bis 0,05 Massenprozent;
Ti in einem Gehalt von mehr als 0 Massenprozent bis 0,05 Massenprozent;
Al in einem Gehalt von 0,01 bis 0,06 Massenprozent;
Cu in einem Gehalt von 0,1 bis 0,6 Massenprozent; und
Ni in einem Gehalt von mehr als 0 Massenprozent bis 0,6 Massenprozent, wobei ein Verhältnis [Ni]/[Cu] des Ni Gehaltes [Ni] zu dem Cu Gehalt [Cu] 0,5 bis weniger als 1,2 beträgt;
gegebenenfalls umfassend Si in einem Gehalt von 0,1 bis 0,6 Massenprozent;
wobei ein Gesamtgehalt von Si und Cu 0,3 Massenprozent oder mehr beträgt, gegebenenfalls umfassend, in chemischer Zusammensetzung, mindestens eines, ausgewählt aus der Gruppe, bestehend aus:
(b) mindestens ein Element, ausgewählt aus der Gruppe, bestehend aus:
V in einem Gehalt von mehr als 0 Massenprozent bis 0,5 Massenprozent;
Cr in einem Gehalt von mehr als 0 Massenprozent bis 1,0 Massenprozent oder weniger; und
Mo in einem Gehalt von mehr als 0 Massenprozent bis 0,5 Massenprozent; und
(c) B in einem Gehalt von mehr als 0 Massenprozent bis 0,005 Massenprozent,
wobei der Rest aus Eisen und unvermeidbaren Verunreinigungen besteht,
wobei eine Mikrostruktur von einer Oberflächenschicht der Stahlplatte mindestens eines von Ferrit und oberem Bainit in einem Gesamtanteil von 80 Flächenprozent bis 100 Flächenprozent umfasst, wie mit dem in der Beschreibung unter der Überschrift "Steel Plate Surface Layer Microstructure" definierten Messverfahren bestimmt,
wobei von der Mikrostruktur der Oberflächenschicht die restliche Mikrostruktur mit Ausnahme des Ferrits und des oberen Bainits gegebenenfalls einen Anteil an Martensit-Austenit-Bestandteil von 0 Flächenprozent bis 5 Flächenprozent aufweist, wie mit dem in der Beschreibung unter der Überschrift "Remainder Microstructure Size" definierten Messverfahren bestimmt,
wobei Körner von dem mindestens einen von Ferrit und oberen Bainit eine wirkliche Korngröße von 2 µm bis 10,0 µm aufweisen, wobei sich die wirkliche Korngröße auf eine durchschnittliche Länge der Körner in Dickenrichtung bezieht, wie mit dem in der Beschreibung unter der Überschrift "Ferrite and Upper Bainite Effective Grain Sizes in Surface Layer" definierten Messverfahren bestimmt,
wobei von der Mikrostruktur der Oberflächenschicht, Körner von einer restlichen Mikrostruktur mit Ausnahme des Ferrits und des oberen Bainits einen durchschnittlichen äquivalenten Kreisdurchmesser von 0,5 µm bis 3,0 µm aufweisen, wie mit dem in der Beschreibung unter der Überschrift "Remainder Microstructure Size" definierten Messverfahren bestimmt, und
wobei die Stahlplatte eine Versetzungsdichte ρ von 5,0× 10¹³ m⁻¹ bis 2,5x 10¹⁵ m⁻¹ aufweist, wie mittels Röntgendiffraktometrie mit dem in der Beschreibung unter der Überschrift "Dislocation Density p" definierten Messverfahren bestimmt.

2. Stahlplatte nach Anspruch 1,
wobei die Stahlplatte eine Bainit-Umwandlungsstarttemperatur Bs von 640°C oder höher aufweist, wobei die Bainit-Umwandlungsstarttemperatur aus der chemischen Zusammensetzung nach Ausdruck (1) berechnet wird: $Bs \left(°C\right) = 830 - 270 \left[C\right] - 90 \left[Mn\right] - 37 \left[Ni\right] - 70 \left[Cr\right] - 83 \left[Mo\right]$ wobei [C], [Mn], [Ni], [Cr] und [Mo] Gehalte von C, Mn, Ni, Cr bzw. Mo (in Massenprozent) darstellen.

## Revendications

1. Plaque d'acier comprenant :
C en une teneur de 0,02 à 0,10 % en masse ;
Mn en une teneur de 1,0 à 2,0 % en masse ;
Nb en une teneur supérieure à 0 % en masse jusqu'à 0,05 % en masse ;
Ti en une teneur supérieure à 0 % en masse jusqu'à 0,05 % en masse ;
Al en une teneur de 0,01 à 0,06 % en masse ;
Cu en une teneur de 0,1 à 0,6 % en masse ; et
Ni en une teneur supérieure à 0 % en masse à 0,6 % en masse, où le rapport [Ni]/[Cu] de la teneur en Ni [Ni] à la teneur en Cu [Cu] est compris entre 0,5 et moins de 1,2 ;
comprenant éventuellement du Si en une teneur de 0,1 à 0,6 % en masse ;
où la teneur totale en Si et Cu est de 0,3 % en masse ou plus,
comprenant éventuellement, en composition chimique, au moins un élément choisi dans le groupe constitué de :
(b) au moins un élément choisi dans le groupe constitué de :
V en une teneur supérieure à 0 % en masse à 0,5 % en masse ;
Cr en une teneur supérieure à 0 % en masse jusqu'à 1,0 % en masse ou moins ; et
Mo en une teneur supérieure à 0 % en masse à 0,5 % en masse ; et
(c) B en une teneur supérieure à 0 % en masse à 0,005 % en masse,
le reste étant constitué de fer et d'impuretés inévitables,
dans laquelle une microstructure d'une couche superficielle de la plaque d'acier comprend au moins un élément parmi la ferrite et la bainite supérieure dans une fraction totale de 80 % de surface à 100 % de surface, telle que déterminée par le procédé de mesure définie dans la description sous le titre « Steel Plate Surface Layer Microstructure » (« Microstructure de couche superficielle de plaque d'acier »),
dans laquelle, parmi la microstructure de la couche superficielle, la microstructure restante, à l'exclusion de la ferrite et de la bainite supérieure, présente éventuellement une fraction de martensite-austénite de 0 % de surface à 5 % de surface, telle que déterminée par le procédé de mesure définie dans la description sous le titre « Remainder Microstructure Size » (« Taille de microstructure restante »),
dans laquelle les grains dudit au moins un élément parmi la ferrite et la bainite supérieure présentent une taille de grain effective de 2 µm à 10,0 µm, où la taille de grain effective se réfère à une longueur moyenne des grains dans le sens de l'épaisseur, telle que déterminée par le procédé de mesure définie dans la description sous le titre « Ferrite and Upper Bainite Effective Grain Sizes in Surface Layer » (« Taille effective de grains de ferrite et de bainite supérieure dans une couche superficielle »),
dans laquelle, parmi la microstructure de la couche superficielle, des grains d'une microstructure restante excluant la ferrite et la bainite supérieure ont un diamètre de cercle équivalent moyen de 0,5 µm à 3,0 µm, tel que déterminé par le procédé de mesure définie dans la description sous le titre « Remainder Microstructure Size » (« Taille de microstructure restante »), et
dans laquelle la plaque d'acier présente une densité de dislocation *ρ* de 5,0 x 10¹³ m⁻¹ à 2,5 x 10¹⁵ m⁻¹, déterminée par diffractométrie aux rayons X avec le procédé de mesure définie dans la description sous le titre « Dislocation Density *ρ* »(« Densité de dislocation *ρ* »).

2. Plaque d'acier selon la revendication 1,
dans laquelle la plaque d'acier a une température de début de transformation de bainite Bs de 640 °C ou plus, où la température de début de transformation de bainite est calculée à partir de la composition chimique selon l'Expression (1) : $Bs \left(°C\right) = 830 - 270 \left[C\right] - 90 \left[Mn\right] - 37 \left[Ni\right] - 70 \left[Cr\right] - 83 \left[Mo\right]$ où [C], [Mn], [Ni], [Cr] et [Mo] représentent les teneurs (en % en masse) respectivement de C, Mn, Ni, Cr, et Mo.
